

Patented Jan. 26, 1926.

1,571,103

# UNITED STATES PATENT OFFICE.

JOSEPH SURY, OF WYNEGHEM, NEAR ANTWERP, BELGIUM.

PHOTOGRAPHIC PIGMENTARY PRINTING PAPER.

No Drawing.

Application filed May 26, 1924. Serial No. 716,049.

To all whom it may concern:

Be it known that I, JOSEPH SURY, a subject of the King of the Belgians, residing at Wyneghem, near Antwerp, in the Kingdom of Belgium, have invented certain new and useful Improvements in Photographic Pigmentary Printing Paper, of which the following is a specification.

The present invention has for its object a photographic paper capable of receiving and retaining, after development, powdered pigments of all colours.

Known pigmentary photographic papers, possess various inconveniences amongst which may be mentioned the absence of visibility of the image after the exposure; the necessity for effecting a transfer on to a provisional support in the case of a paper having a thick emulsion and on the other hand the necessity for great exactness in working in the case of a paper having a thin emulsion to avoid producing excessive insolubility of the blacks.

The purpose of the present invention is to remedy these inconveniences that is to say to provide a pigmentary paper giving a visible picture at the time of exposure consequently not necessitating the use of a photometer, the said paper being developed without previous transfer and being capable of receiving and retaining after development, powdered pigments of all colours.

The improved paper is manufactured by incorporating with a colloidal emulsion a temporary colouring matter serving as guide for developing, said colouring matter being permeable to light and capable of dissolving easily in a diluted acid while producing a gas which by its discharge imparts to the gelatinous layer of colloid emulsion a spongy property enabling it to retain in its pores powdered pigments ultimately applied on its surface.

In the practical working of the invention the temporary colouring matter permeable to light and consequently having to be of a blue colour, is composed of aluminum sodium silicate and sodium pentasulfid.

This colouring matter is mixed with a certain quantity of a powdered inert white substance, for instance barium sulfate, kaolin, or the like, which, incorporated with the colloidal emulsion, prevents contraction or sinking of the moist emulsion after the disappearance of the blue colouring matter so as to form as it were infinitesimal pillars

and arches which during the drying maintain open the microscopic cavities produced by the disappearance of the colouring matter and the gaseous discharge.

In order to carry out the invention a paper preferably thickly sized, is coated with an emulsion of one or more colloids, for instance gelatine, gum arabic, albumen, or a mixture of these substances in which has been incorporated a certain quantity of powdered barium sulfate or kaolin to which is added aluminum sodium silicate and sodium pentasulfid.

This mixture is spread by any means over the non-porous surface of the paper and is allowed to dry.

When the paper is required for use it is sensitised by means of an aqueous or aqueo-alcoholic solution of an alkali bichromate.

After drying the paper is exposed under a negative and the resulting print can be inspected owing to the appearance of the image resulting from the action of the light on the bichromate. After printing the picture is developed in cold or hot water then decoloured in a diluted solution of hydrochloric acid. Under the action of this bath, the blue colouring matter dissolves with gaseous production of hydrogen sulfid and sulphurous acid. This gaseous discharge by producing an effervescence renders the layer of pasty colloidal emulsion spongy the barium sulfate (or the kaolin) contained in the emulsion being present therein in the form of infinitesimal pillars and arches keeping open, during drying, the microscopic cavities produced by the disappearance of the colouring matter and the gaseous effervescence as previously described.

After drying, the emulsion which coats the paper is capable owing to its porosity of retaining any powdered pigment applied on its surface. This pigment not being fixed by an adhesive can be transferred by slight pressure on to a sheet of paper coated with an adhesive or the pigment can be fixed on the original print similarly to fixing a charcoal drawing.

Alternatively the dried porous emulsion, when pressed hard against a plate of sufficiently soft metal will produce on the metal plate an etching capable of being inked with fatty inks and a number of copies can be printed therefrom by means of a printing press.

The improved paper has not only the ad-

vantage of allowing the exposure to be gauged owing to the visibility of the image, thus rendering the use of a photometer unnecessary, but further allows an easy transfer of the image which is particularly advantageous in colour photography wherein three selected colour images (yellow, red, blue) are superposed by transfer method on to a support to reproduce the natural colours 10 of the object photographed.

What I claim is:

1. A pigmentary photographic printing paper, characterized by a colloidal coating, containing a temporary colouring matter 15 permeable to light and capable of being dissolved by a diluted acid with gaseous dis-

charge whereby the colloidal coating is rendered spongy.

2. A pigmentary paper, as in claim 1, wherein the temporary colouring matter is 20 composed of aluminum sodium silicate and sodium pentasulphide mixed with a powdered inert white substance, whereby to provide means for keeping open the cavities produced in the colloidal coating by the dissolving of the colouring matter and the 25 gaseous discharge produced by a solution of hydrochloric acid.

In testimony whereof I have affixed my signature.

JOSEPH SURY.